

June 22, 1926.

1,589,365

P. C. CHESTERFIELD

MOLD FOR CASTING METAL

Filed March 22, 1923

2 Sheets-Sheet 1



Witnesses

H. G. Marks  
James Celano

By

Inventor  
PERCY C. CHESTERFIELD  
Charlottesville

Atty.

June 22, 1926.

1,589,365

P. C. CHESTERFIELD

MOLD FOR CASTING METAL

Filed March 22, 1923

2 Sheets-Sheet 2



Witnesses

Al Darks  
James Celano

by

Inventor

PERCY C. CHESTERFIELD  
Charlton Hills

Atty

Patented June 22, 1926.

## UNITED STATES PATENT OFFICE.

PERCY C. CHESTERFIELD, OF DETROIT, MICHIGAN, ASSIGNOR TO CHESTERFIELD METAL COMPANY, OF DETROIT, MICHIGAN, A CORPORATION OF MICHIGAN.

## MOLD FOR CASTING METAL.

Application filed March 22, 1923. Serial No. 626,801.

- This invention relates to improvements in methods of casting alloys and molds therefor, and, while not restricted to such use, are especially adapted for 5 the manufacture of cutting tools of self-hardening alloys, such as those composed of both cobalt and nickel or one of these metals singly and one or more members of the chromium group.
- 10 One of the principal objects of my invention is the provision of means whereby the hardness of the resulting casting is maintained substantially uniform in spite of variations in the rate of solidification and cooling of the metal.
- 15 A further object of the invention is the provision of an improved form of mold for producing castings of metal which shrink on solidification.
- 20 It is also an object of the invention to provide a simple form of mold for casting metal.
- 25 Other and further important objects of this invention will be apparent from the disclosures in the following specification.
- On the drawings:
- Figure 1 is a side elevation of a battery of molds embodying the present improvements.
- 30 Figure 2 is a section on the line 2—2 of Figure 1.
- Figure 3 is a cross-section through an individual mold after the metal has been cast.
- Figure 4 is a front elevation of one half 35 of a modified form of mold.
- Figure 5 is a section on the line 5—5 of Figure 4.
- The apparatus comprises a frame to carry a battery of molds for the metal to be cast.
- 40 The frame consists of a pair of end plates 5 secured in spaced relation by stays 6 and a pair of bars or tubes 7 which act as the supports for the molds.
- The molds are preferably made of graphite 45 slabs 8 and 9. These slabs are cut away at one end and in the cut away portion of one slab (as 8) is secured a cross piece of graphite 10 adapted to enter the corresponding recess in the other slab. This cross piece may conveniently be held in position 50 by wood screws 11 and also by a suitable cement such as a mixture of sodium silicate solution and graphite.
- In the abutting faces of the slabs are cut 55 grooves 12 of triangular section extending
- from the top of the slab to the cut-away portions or recesses in the bottom thereof. Further above the recesses cross grooves 13 are formed. These grooves are conveniently formed prior to the securing of the cross 60 piece 10 in position.
- When the two slabs are brought together, a series of vertical channels are formed connected together at their lower ends so that if molten metal be poured down the middle 65 channel it will enter and rise up the side channels so that five (or more) bars may be cast simultaneously.
- The metal for which this mold was particularly designed shrinks on solidifying so 70 that the grooves are made triangular as shown to provide wedge surfaces between the cast metal and the mold which enables the former to push the two halves of the latter apart as the metal shrinks.
- 75 The frame which carries these molds is designed to allow the two halves of the molds to separate in this way. Thus, resting on the pipes 7 are a pair of plates 14 apertured for the passage of the stays 6. 80 On the latter are arranged springs 15 adapted to press the plates 14 towards the series of molds arranged therebetween.
- The pressure exerted on the molds by 85 these springs may be adjusted by means of a further plate 16, also slidable on the stays 6, against one side of which one set of springs 15 bear and against the other side of which bears the screw 17. This screw 17 and plate 16 also enable the apparatus 90 to be used with a varying number of molds, as desired.
- While these molds are preferably constructed of graphite, they may also be made of cast iron, in which case the molds are 95 treated before use with a solution of sulphuric acid to prevent the hot metal adhering thereto.
- Graphite is, however, much superior to cast iron as a material for molds. In 100 the first place it is much easier to machine graphite than cast iron so that molds for casting special sizes and shapes can be more readily made. Then again, cast iron molds have to be repeatedly treated with sulphuric acid solution since the effect of the treatment soon wears off.
- Further, cast iron molds, especially for 105 small sizes of bars, chills the metal too rapidly. This chilling makes the bars hard 110

and, while hardness is a desideratum, it should be uniform throughout the bar and chilling makes the outer layers harder than the center.

5 Now graphite has a lower specific heat per unit volume than cast iron, being only 65% of that of the latter material. Further, the heat conductivity of graphite is only 11% of the heat conductivity of cast iron. 10 Consequently the rate of abstraction of heat from the cooling metal is far less in the case of graphite than in the case of cast iron molds.

Graphite has the additional advantage of 15 giving a very smooth surface—a most important desideratum in the casting of self-hardening alloys, as the only way the latter can be worked after casting is by grinding and this is a slow operation in view of the 20 extreme hardness of the alloys.

Where elasticity in the mold is required, as where rings have to be cast and the core must compress to allow for the contraction of the parts, graphite is especially useful.

25 Where sand molds are used, even if brushed over with graphite powder, the bars are full of blow holes and the metal is too soft for use as a high-speed lathe tool.

Whether the molds are made of graphite 30 or cast iron, they should be warmed before use, and for this purpose a series of gas jets 18 are arranged beneath the molds. To conserve the heat of these jets, a hood 19 may conveniently be used to cover the apparatus while it is being warmed prior to 35 use and then removed by handle 20 for the casting operation.

Above the central channel of each mold 40 a gate 21 is placed to act as a funnel for the cast metal. These gates, which may conveniently be made of cast iron, are made in two halves detachably held together by clips 22.

The mold shown in Figures 4 and 5 is 45 adapted for casting rings. In this case one half 25 of the mold is formed with a circular recess 26 having a shoulder 27 formed therein for engagement with the periphery of an annular core 28. This core is cut 50 diagonally, as at 29, like a piston ring, so that as the metal cools the ring may compress and close this slot.

The other half of the mold is a plain 55 slab of graphite 29 adapted to seal the annular space around the core 28. A groove 30 is formed in the half-mold 25 for the passage of the molten metal into such annular space, and a groove 31 for the escape of air therefrom. In connection with these 60 molds, as in the previous forms, a casting gate 32 is provided.

By this construction a ring may be cast 65 having a cylindrical inner surface. If the core were not compressible, it would be necessary to make the core conical to allow

the shrinking metal an opportunity to push the two parts of the mold apart against the action of springs. With the construction shown the two halves of the mold may be firmly clamped together.

70 After the castings have cooled the two halves of the mold are separated and the casting taken out. In the case of bars these are all connected at their lower ends and this connecting piece, as well as the metal which extends up through the casting gate, 75 has to be cut off. For this purpose a cutting-off wheel of carborundum or the like may be used. After a nick has been cut in each side the intervening metal is fractured 80 by a sharp blow with a hammer. The bars are then smoothed and ground to the desired form by carborundum or other abrasive wheels.

The alloy for which the above mold is 85 more particularly designed is one comprising cobalt and/or nickel and one or more of the metals of the chromium group.

A suitable alloy is one whose metallic components consist of:

|          | Per cent. |
|----------|-----------|
| Nickel   | 14        |
| Cobalt   | 27        |
| Chromium | 31        |
| Tungsten | 28 95     |

To the above constituents is added a hardening element, such as carbon, either free or as a carbide.

Certain of the carbides are excessively hard, for example, boron carbide and titanium carbide are the only two substances known at present which are hard enough to cut diamond. Similarly, silicon carbide and tungsten carbide are sufficiently hard to scratch corundum, while chromium carbide 100 will scratch topaz.

I have found that additions of boron carbide and titanium carbide give better and more uniform results than carbon alone, and preferably, therefore, I use one or other, 110 or possibly both, of these two substances or any other carbide which may be found hereafter having a greater hardness than silicon carbide. Silicon may also be used in some cases, added either in the free state or as the 115 carbide.

I have also found that the hardness of bars cast from the above alloy vary according to the rate at which they cool so that a small bar, which necessarily cools more 120 rapidly than a large one, is, other conditions being the same, harder. On the other hand, increasing the carbon content of the alloy increases its hardness. It has further been found that heat treatment of the alloy after 125 casting does not appreciably change the hardness so that the alloy may be termed "self-hardening."

To secure the best results it is necessary to hit the happy mean between too great 130

hardness, which means brittleness, and liability to flake or chip, and too little hardness, which means that a tool made therefrom will be too soft to cut for the desired length of time or to cut hard metals.

5 This I accomplish by the present invention by varying the amount of hardening element, such as boron carbide, added with varying dimensions of the bar to be cast.

10 For example, for a  $\frac{1}{4}$  inch bar 0.56% boron carbide may be used to advantage; for a  $\frac{3}{8}$  inch bar 0.85%; and for a  $\frac{1}{2}$  inch bar 0.97%.

15 By so varying the content of boron carbide the sum of the hardness due to chilling and the hardness due to the hardening element is maintained substantially uniform irrespective of the size of the bar cast.

20 In addition to the carbon added, as boron carbide, there is also a certain carbon content in the constituent metals and a further small quantity of carbon is picked up from the crucible if an unlined graphite crucible be employed.

25 As a result of the picking up of carbon from the crucible, it is desirable to avoid heating the metal too much or too long in the crucible, and further, when remelting scrap along with a proportion of new metal, to reduce the amount of boron carbide added to carbonize the latter.

I claim as my invention:

30 1. A mold for casting metal comprising a pair of uprights, a pair of rods connecting the upper portions of said uprights, a second pair of rods connecting the lower portions of said uprights, a mold comprising two vertical sections adapted to slide vertically between the first pair of rods and to rest upon the second pair of rods and releasable means for holding the two sections of the mold together.

35 2. A mold for casting metal comprising a pair of uprights, pairs of rods connecting the upper and lower portions of said uprights, a mold comprising two vertical sections between said uprights, means for supporting said mold, a plate having apertures for the passage of said rods and slidable thereon adapted to engage one section of said mold, a second plate having apertures for the passage of said rods and slidable there-

on, coiled springs around each of said rods between said plates and means for adjusting the position of the second plate to the adjacent upright.

40 3. A mold for casting metal comprising a pair of uprights, pairs of rods connecting the upper and lower portions of said uprights, a mold comprising two vertical sections adapted to slide vertically between said pairs of rods, a further pair of rods between said uprights below and between the lowermost of the first mentioned pairs of rods for supporting the mold, a plate having apertures for the passage of said rods and slidable thereon adapted to engage one section of said mold, a second plate having apertures for the passage of said rods and slidable thereon, coiled springs around each of said rods between said plates and means for adjusting the position of the second plate to the adjacent upright.

45 4. A mold for casting metal comprising a pair of uprights, rods connecting said uprights, means for supporting a mold comprising two vertical sections between said uprights, a pair of plates slidable upon said rods, one of said plates contacting springs on said rods between said plates, and means for adjusting the position of the other plate relatively to the upright adjacent thereto.

50 5. A mold for casting metal comprising a pair of graphite slabs, each of said slabs being recessed at one end, a strip of graphite arranged in the recess of one slab and secured thereto and adapted to enter the corresponding recess in the other slab, and a longitudinal groove in one slab for the reception of the metal to be cast.

55 6. A mold for casting metal comprising a pair of plates, one of the plates having an offset portion adapted to enter a recess in the other plate, said last mentioned plate having a groove therein extending transversely with respect to the offset portion for the reception of the metal to be cast, said groove extending to said recess and being closed at its lower end by said offset portion when the plates are in engagement with each other.

In testimony whereof I have hereunto subscribed my name.

PERCY C. CHESTERFIELD.